

## UNITED STATES PATENT OFFICE

2,427,034

CERAMIC COMPOSITION FOR AIRCRAFT  
SPARK PLUGS

Eugene Wainer, Niagara Falls, N. Y., assignor to  
The Titanium Alloy Manufacturing Company,  
New York, N. Y., a corporation of Maine

No Drawing. Application March 18, 1942,  
Serial No. 435,130

5 Claims. (Cl. 106—57)

1

This invention relates to electrically insulating refractory compositions resistant to corrosion by gasoline fuels containing lead oxide. More particularly, it relates to such compositions which are suitable for use as ceramic insulators for spark plugs in aircraft engines and similar high compression internal combustion engines where gasoline containing lead compounds are used.

Ceramic insulators for automotive spark plugs have been extensively used for many years. Generally, the type of ceramic compositions used in automobile internal combustion engines also serve fairly well for aircraft engine use, as long as they are used in low power, low compression, and low speed engines. However, in recent years the horsepower output per unit weight of aircraft engines has been greatly increased, with the result that the motors operate at considerably higher temperatures, higher speeds and higher compressions. Under these conditions, the usual type plugs become less and less useful. Coincidental with the development of more highly powered engines, the elimination of piston knock by means of gasolines treated with tetra-ethyl lead has introduced further problems of such a nature as to render an automotive spark plug useless in the modern aircraft engine. For example, when the full power of a 1000 horsepower aircraft engine is suddenly developed, as in quick take offs or rapid climbs, temperatures up to 1800° F. are developed in the vicinity of the ceramic insulator used in the plug. At the same time the lead compound in the anti-knock gasolines decomposes to lead oxide, which deposits on the red hot ceramic insulator, with the result that extremely corrosive conditions are obtained. Under such conditions, the usual automotive plug is destroyed for all practical purposes in a very few minutes.

For the above reasons, ceramic compositions having highly unusual properties are required for satisfactory service as spark plug insulators in the modern aircraft engine. Of these unusual properties, one of the most important is the necessity for complete resistance to corrosion by molten lead oxide. This property is normally evaluated by immersing the suitably prepared composition in molten litharge at 1800° F. for a period of 24 hours. Compositions showing 5% or less volume decrease under such a test are considered suitable. Besides this property, the body must be an electrical insulator at elevated temperatures. It must be capable of vitrification at commercially obtainable temperatures (i. e., its "maturation temperature" must not be too high), and must have high thermal conductivity, high

5 mechanical strength, and high resistance to thermal shock. Finally, the composition must be refractory in nature, that is it must not melt or decompose at the high temperatures encountered in aircraft engines.

In accordance with this invention, compositions have been developed which admirably fulfill these requirements. Such compositions comprise fired mixtures of zirconium oxide and magnesium oxide, in proportions ranging from one mol of zirconia to two mols of magnesia, to two mols of zirconia to one mol of magnesia. In such compositions the zirconia and magnesia together, and usually the zirconia alone, comprise at least 10 50 per cent of the dry composition, even when other ingredients are present. For compositions containing less magnesium oxide than a 1:1 molar ratio, the silica content should be as low as possible, while at ratios of 1:1 or higher, silica up to 15 20 10% of the total may be included without materially affecting the lead resistance.

Since combinations of zirconia and magnesia have proved so successful, combinations of zirconia with other group II oxides, such as oxides 25 of beryllium, calcium, strontium, barium and zinc were also tried, without magnesia, but unsuccessfully. For example, among other disadvantages, combinations of zirconia with calcium oxide, strontium oxide or barium oxide require 30 such exacting control of the firing temperature as to be commercially impracticable. Beryllium oxide is too costly for commercial use, and also requires a higher temperature to fire or mature the bodies (maturation temperature) without any 35 compensating advantage. Combinations of zinc oxide with zirconia alone have too short a firing range. However, under certain conditions, the addition of small amounts of other group II oxides, particularly barium and zinc, to the magnesia-zirconia combinations has been found to 40 45 be beneficial in reducing maturation temperatures. In addition, the presence of zinc oxide appears to markedly reduce the wettability of the ceramic composition by molten lead oxide. In any case, the molal percentage of any of these other group II oxides should always be less than either the magnesia or zirconia.

Besides the essential ingredients zirconium oxide and magnesium oxide, there may also be 50 present a certain amount of silica. Its presence in the compositions has several decided effects, some beneficial and some detrimental, so that the permissible amount of silica is quite critical. Thus, it increases the mechanical strength of the fired body, while relatively small quantities

markedly reduce reaction and maturation temperatures. By its use, a considerably tighter degree of vitrification is obtainable at a lower temperature than otherwise. At the same time the use of silica in the composition seriously affects the general lead oxide resistance of the finished body. In general, as low a silica content as possible should be present when the molar ratio of magnesia to zirconia is less than 1:1, and the silica should not be more than 10% by weight of the composition in any case. It is preferred that the higher silica contents be used only with a 2 to 1 ratio of magnesia to zirconia.

Under certain conditions, the presence of alumina in the composition is desirable. Like silica, it aids in increasing the mechanical strength of the body. In addition, it does not seem to be harmful as far as resistance to corrosion by lead oxide is concerned. It does, however, considerably increase maturation temperatures. The result is that not more than 25% alumina should be present, if silica is present, and not more than 10%, if silica is absent.

Although combinations of zirconia and magnesia with small amounts of other oxides ( $Al_2O_3$ ,  $SiO_2$  and group II oxides) may be used, it is preferred to use combinations of pure zirconia and magnesia for use in spark plugs. Since electrical resistance is important, alkali metal compounds and heavy metal compounds, such as iron and manganese, should be kept to a minimum. In any case, the total amount of these impurities in the composition should be less than 1 percent.

The compositions of the present invention are prepared by calcination of mixtures of the finely divided oxides, or of compounds which form the oxides at elevated temperatures, such as carbonates and the like. Soluble salts other than the halides may be used as starting materials except in the case of barium and strontium. Where these elements are present, the sulfate radical should not be present due to the sluggishness with which sulfur is eliminated on calcination. Any pure form of zirconium oxide or other zirconium compound forming zirconium oxide at elevated temperatures may be used as a starting material. Particularly suitable (except of course where barium or strontium is present) are the water insoluble oxysulfates of zirconium described in copending applications Serial Nos. 404,875 and 404,876, because of their high purity and the state of subdivision and reactivity these materials afford. To react suitably, the initial zirconium oxide preferably should have an average particle size of 1 micron or less, or the initial material should be a compound of such nature that on calcination a zirconia of particle size 1 micron or less is obtained. Zirconium oxysulfate is particularly suitable because on calcination to the oxide a particle size of 0.1 to 0.2 microns can be obtained.

The suitably compounded mixtures are prepared by calcination to 2400 to 2600° F. until reaction is complete. Normally, an easily disintegrable calcine is obtained. The calcine is comminuted to pass a 200 mesh screen and is then formed by a variety of procedures into the necessary shapes. The compositions may be pressed, rammed, jiggered, extruded or slip cast. Pressing or ramming can be done with the addition of a water solution of dextrine, gelatine or similar organic bonding agent to yield the necessary green strength. Casting or jiggering forming is done by means of additions of minute quantities of

modifiers or agents which liquefy or deflocculate the slip. Such modifiers may be sodium silicate, or more preferably any of those described in copending applications Serial Nos. 330,373 and 427-5281. In casting, enough water is added to form a fluid slip, while in jiggering the same agents are added plus enough water to yield a dough. In jiggering, tempering of the body is usually aided by the addition of a small amount of acid, preferably organic in nature, such as oxalic acid, this being particularly useful when the body is to be extruded. In adding oxalic acid as a tempering agent, the deflocculants and water are added first, and the oxalic acid is then added to the thoroughly mixed batch. An amount of deflocculating agent equivalent to 0.05 to 0.5% of the batch is sufficient for casting, and the acid addition for extrusion or jiggering is 0.1 to 1.0%.

After forming and shaping, the body is dried and fired in a clean oxidizing atmosphere to maturation. For the bodies described above, in no case does the maturation temperature exceed 3100° F. Finally, the material is polished to form the ceramic for spark plug insulators.

The invention having been described, the following examples will point out specific methods of practicing the same:

*Example 1*

30. 192 grams of basic magnesium carbonate containing 42.0%  $MgO$  is thoroughly mixed with 200 grams of dry zirconium oxysulfate containing 61.5%  $ZrO_2$ . The mixture is calcined at 2600° F. for three hours. It is then disintegrated by passage through a high speed swing hammer mill. The calcine is then prepared for slip casting as follows: 100 grams is mixed with 22 cc. of water to which is added 0.07 gram of  $Na_4P_2O_7$ . After casting in plaster of Paris molds, the piece is removed and dried and fired to 3050° F. in three hours, maintained at peak temperature for 1½ to 2 hours, and then cooled.

The same calcine can be used for jiggering or extrusion by mixing 100 grams of the powder with 15 to 19 cc. of water to which 0.05 gram of  $Na_4P_2O_7$  has been added. After thorough mixing, 0.1 gram of finely powdered oxalic acid is completely kneaded in and the doughlike mass then worked into shape. The mass is dried and fired as above.

*Example 2*

192 grams of basic magnesium carbonate and 200 grams of zirconium oxysulfate as in Example 1 is thoroughly mixed with the addition of 6 to 16 grams of -325 mesh silica, preferably of the flour type. The same procedure is followed as in Example 1, except that the presence of the silica enables the calcination temperature of the composition to be lowered 50 to 150 degrees, and the maturation temperature 50 to 150 degrees, depending on the quantity of silica. The body may be prepared for slip casting as follows: 100 grams of calcine is mixed with 20.0 cc. of water, 0.1 gram of  $NH_4OH$  and 0.1 gram of tannic acid. This mixture is suitable for plaster mold casting. The mix may be extended or jiggered by reducing the initial water to 15 cc., mixing thoroughly, and adding 0.2 gram of powdered oxalic acid and kneading thoroughly.

*Example 3*

80.6 grams of -325 mesh  $MgO$  (prepared from calcination of the precipitated carbonate) plus 75. 123 grams of  $ZrO_2$  (prepared by low temperature

calcination of zirconium carbide or cyanonitride) are mixed with 20 grams of silica flour and 15 grams of light grade aluminum hydrate containing 65%  $\text{Al}_2\text{O}_3$ . The mixture is calcined at 2400° F. for three hours. On cooling, the disintegrated calcine is formed by pressing from a mixture containing 100 grams of calcine and 12 cc. of 1% gelatine solution. The body is fired to 2850 to 2900° F. for maturation and vitrification.

*Example 4*

96 grams of basic magnesium carbonate and 200 grams of zirconium oxysulfate as in Example 1 are mixed with 6.0 grams of Georgia kaolin plus 5 grams of silica flour. This mixture is calcined at 2400° F., formed and shaped as in any of the preceding examples, and fired at 2900° to 2950° F. for maturation.

*Example 5*

41 grams of -325 mesh pure  $\text{MgO}$  and 123 grams of  $\text{ZrO}_2$  (formed by calcination of zirconium oxysulfate at 1600° F.) are mixed with 13 grams of precipitated  $\text{BaCO}_3$  and 3.5 grams of silica flour. In place of  $\text{BaCO}_3$ , 6.5 grams of precipitated  $\text{CaCO}_3$  or 9.7 grams of  $\text{SrCO}_3$  may be used. The mixture is calcined at 2400° F., formed and shaped as in any of the preceding examples, and fired at 2850° F. for maturation.

*Example 6*

41 grams of -325 mesh pure  $\text{MgO}$  is mixed with 123 grams of  $\text{ZrO}_2$  (formed by calcination of pure zirconium carbide or cyanonitride). To this is added either 13 grams of precipitated  $\text{BaCO}_3$ , or 6.5 grams of precipitated  $\text{CaCO}_3$  or 9.7 grams of precipitated  $\text{SrCO}_3$ . 4 grams of zinc oxide and 3.5 grams of silica flour are then added, the composition mixed thoroughly and calcined to 2400° F., for reaction. The calcine is shaped and formed as in any of the preceding examples, and then matured at about 2800-2850° F. This body has a short firing range between maturation and plastic flow.

*Example 7*

41 grams of -325 mesh  $\text{MgO}$  and 123 grams of pure  $\text{ZrO}_2$  are mixed with 20 grams of  $\text{BaCO}_3$  and calcined to 2450° F. for reaction. Maturation takes place at 2800 to 2850° F.

*Example 8*

41 grams of  $\text{MgO}$  plus 123 grams of  $\text{ZrO}_2$  plus 13 grams of  $\text{BaCO}_3$  plus 7.5 grams of aluminum hydrate plus 5 grams of silica flour are mixed together and calcined to 2400° F. for reaction. The body matures at 2800° F.

In addition to use in aircraft and similar high compression internal combustion engines, the ceramic compositions of the present invention may be used in forming containers for the fusion of lead and its alloys, for which suitable containers have always been a problem when the temperatures exceed the melting point of lead by a few hundred degrees. Furthermore, since

the electrical resistance is relatively high at elevated temperatures, and since the thermal conductivity at such temperatures is also high, the compositions are also useful for the embedding or packing of resistance wires in the assembly of electric cooking range elements, hot plates, soldering irons and the like.

When parts or percentages are mentioned, parts and percentages by weight are understood.

10 As many variations are possible within the scope of this invention, it is not intended to be limited except as defined by the appended claims.

I claim:

15 1. A spark plug having a ceramic insulator comprising a fired mixture containing a major proportion of zirconium oxide plus magnesium oxide, the molal proportion of zirconium oxide to magnesium oxide being between 2 to 1 and 1 to 2.

20 2. A spark plug having a ceramic insulator comprising a fired mixture containing a major proportion of zirconium oxide plus magnesium oxide, the molal proportion of zirconium oxide to magnesium oxide being between 2 to 1 and 1 to 2, said composition containing less than 10 per cent silica and less than 25 per cent alumina.

25 3. A spark plug having a ceramic insulator comprising a fired mixture containing a major proportion of zirconium oxide plus magnesium oxide, the molal proportion of zirconium oxide to magnesium oxide being between 2 to 1 and 1 to 2, said composition containing less than 10 per cent barium oxide.

30 4. A spark plug having a ceramic insulator comprising a fired mixture containing a major proportion of zirconium oxide plus magnesium oxide, the molal proportion of zirconium oxide to magnesium oxide being between 2 to 1 and 1 to 2, said composition containing less than 10 per cent zinc oxide.

35 5. The method of forming an insulator body for spark plugs, comprising forming a mixture of zirconium oxysulfate and magnesium carbonate, the proportion of zirconia to magnesia in said mixture being between 2 to 1 and 1 to 2, calcining said mixture, forming said calcined mixture into shape, drying and firing to vitrification.

EUGENE WAINER.

50 REFERENCES CITED

The following references are of record in the file of this patent:

55 UNITED STATES PATENTS

| Number    | Name           | Date           |
|-----------|----------------|----------------|
| 1,682,251 | Riddle         | Aug. 28, 1928  |
| 1,324,546 | Ferngren       | Dec. 9, 1919   |
| 1,728,748 | D'Ans          | Sept. 17, 1929 |
| 1,818,903 | Martin         | Aug. 11, 1931  |
| 2,040,215 | Rava           | May 12, 1936   |
| 2,172,839 | Francis et al. | Sept. 12, 1939 |
| 2,098,812 | Pulfrich       | Nov. 9, 1937   |
| 1,418,372 | French         | June 6, 1922   |